

July 2, 1963

R. B. PUYEAR

3,096,160

VAPOR DIFFUSION COATING PROCESS

Filed June 19, 1961

2 Sheets-Sheet 1

*Fig. 1.*



*Fig. 2.*



INVENTOR.  
ROBERT B. PUYEAR

BY

Her A. Plum, Jr.

ATTORNEY

July 2, 1963

R. B. PUYEAR

3,096,160

VAPOR DIFFUSION COATING PROCESS

Filed June 19, 1961

2 Sheets-Sheet 2

*Fig. 3.*



*Fig. 4.*



INVENTOR.  
ROBERT B. PUYEAR

BY

Leo A. Plum, Jr.

ATTORNEY

# United States Patent Office

3,096,160

Patented July 2, 1963

1

3,096,160

VAPOR DIFFUSION COATING PROCESS  
Robert B. Puyear, Kokomo, Ind., assignor to Union Carbide Corporation, a corporation of New York  
Filed June 19, 1961, Ser. No. 117,974  
16 Claims. (Cl. 29—197)

This invention relates to the application of diffused metallic coatings to metal articles.

Engineering parts subjected to high temperatures and corrosive atmospheres can often be made more resistant to these forces by the application of a protective surface coating to the part. The protective coating composition is selected to give increased resistance to those forces which attack the surfaces of an article, namely oxidation, corrosion, and erosion, just as proper metallurgical design selects the alloy base of the article on the basis of its tensile and creep strengths. Additionally the coating must be adherent and ductile enough to permit the intended use of the coated part without danger of spalling or chipping of the coating. Cementation processes such as chromizing and calorizing produce coatings of chromium and aluminum, respectively, which are resistant but which often have a brittle bonding layer with the base metal.

Protective coatings composed of alloys are very desirable, in view of the superior properties possessed by many alloys over the elemental metals. Of exceptional utility as a protective coating would be a diffusion coating of certain aluminum-containing alloys and/or intermetallic compounds of iron and cobalt which are reported to possess exceptional oxidation resistance as well as the ductility and strength needed for a good bond. These materials further possess a resistance to high temperatures greater than that of the individual constituents of the materials.

Present methods for producing alloy coatings on metallic articles generally require a multiple step operation with a coating of one metal followed by the coating with the other metal, and then a heating to achieve the alloying. Such processes are complicated and unwieldy, and do not consistently yield the desired coating composition or thickness. It is especially difficult to coat articles having complex shapes by electrodeposition. The part of the article nearest the sacrificial electrode receives the heaviest coating and the crevices, internal cavities, and corners receive little or no coating.

It is the primary object of this invention, therefore, to provide compositions and methods for producing adherent diffusion coatings of high temperature resistant aluminum alloys.

It is another object of this invention to provide a method for applying aluminum alloy diffusion coatings on metallic articles which method is simple and requires a minimum of steps.

2

It is also an object of this invention to provide an aluminum alloy diffusion coating for metallic articles giving maximum oxidation and erosion resistance to the coated article, thereby allowing its use in more stringent applications than ordinarily possible.

Other aims and advantages of the invention will be apparent from the following description and the appended claims.

In accordance with these objects a process for diffusion coating metallic articles is provided comprising embedding an article to be coated in particulated, prealloyed charge material consisting essentially of from about 19 percent to about 35 percent by weight aluminum and the balance at least one metal selected from the group consisting of iron and cobalt and incidental impurities, and heating said charge and contained articles in the presence of at least one material selected from the group consisting of ammonium halides and aluminum halides, said heating being conducted with the exclusion of air at a temperature between about 1400° F. and 2000° C. for a time sufficient to form a coating.

In the drawings:

FIG. 1 is a cross-section, magnified 500 times, of the diffused coating produced on a cobalt-base article by the process of this invention;

FIG. 2 is a schematic representation of a reaction chamber or retort for containing the charge material, articles to be coated, and carrier material according to the process of this invention;

FIG. 3 is a cross-section, magnified 150 times, of the diffused coating produced on an iron-base alloy by the process of this invention;

FIG. 4 is a cross-section, magnified 150 times, of the diffused coating produced on the iron-base article of FIG. 3 but with another coating thickness.

Articles that can be coated according to this process include alloys having a base of a metal selected from the group consisting of iron, nickel, cobalt, and copper.

Preferably the articles to be coated are selected from those iron-base, nickel-base, cobalt-base and copper-base alloys which contain a predominant amount of the base metal. In this regard, predominant means possessing that minimum amount of iron, nickel, cobalt or copper which will result in the superior coating thickness and characteristics shown in the drawings and the examples following. As used herein, the term "alloys" is meant to include the pure or substantially pure metal itself, i.e. iron, nickel, cobalt or copper articles.

In Table 1 are shown a number of representative metals and alloys which were satisfactorily coated by the process of this invention. The compositions do not show the carbon content or other minor constituents, except that manganese and silicon contents are shown for the iron-base alloys.

TABLE 1

Nominal Composition of Metals and Alloys Coated

| Alloy No.         | Ni   | Co  | Fe  | Mo  | Cr   | W    | Mn  | Si  | Others   | Form     |
|-------------------|------|-----|-----|-----|------|------|-----|-----|----------|----------|
| Iron-base Alloys: |      |     |     |     |      |      |     |     |          |          |
| F1                |      |     | 99+ |     | 8.5  |      |     | 3.5 |          | Wrought. |
| F2                |      |     | 87  |     | 16.0 |      | .5  |     | 3.25 Cu. | Cast.    |
| F3                | 4.1  |     | 75  |     | 21   |      | 9   |     |          | Do.      |
| F4                | 4    |     | 65  |     | 19   |      | 1   | 3.0 |          | Do.      |
| F5                | 8    |     | 69  |     | .2   | .5   | .8  | .3  |          | Do.      |
| F6                | .5   |     | 97  |     | 3.0  | 19.0 | 1.5 | .7  |          | Do.      |
| F7                | 13.0 |     | 52  |     | 24.0 |      | .9  |     |          | Do.      |
| F8                | 20.5 |     | 54  |     | 17   |      | 1.5 |     |          | Do.      |
| F9                | 12   |     | 67  | 2.5 |      |      |     |     |          | Wrought. |
| F10               |      |     | 86  |     | 12.5 |      | .8  |     |          | Do.      |
| F10A              |      |     | 85  |     | 12.5 |      | .8  | .4  |          | Cast.    |
| F11               |      |     | 82  |     | 16   |      | 1.5 |     |          | Wrought. |
| F12               | 9    |     | 73  |     | 18   |      |     |     |          | Cast.    |
| F13               |      | 6.3 | 61  | 16  | 17   |      |     |     |          | Do.      |

TABLE 1—Continued  
Nominal Composition of Metals and Alloys Coated

| Alloy No.           | Ni   | Co | Fe  | Mo  | Cr   | W    | Mn  | Si  | Others    | Form     |
|---------------------|------|----|-----|-----|------|------|-----|-----|-----------|----------|
| F14                 | 20   | 19 | 35  | 3   | 21   | —    | —   | —   | —         | Wrought. |
| F15                 | .5   | —  | 97  | .2  | 5    | —    | 8   | 3   | —         | Do.      |
| F16                 | .4   | —  | 87  | —   | 8.5  | —    | 4   | 3.3 | —         | Do.      |
| F17                 | 1.8  | —  | 75  | —   | 20   | —    | 4   | 2.4 | —         | Do.      |
| F18                 | 12.0 | —  | 67  | —   | 18.8 | —    | 1.5 | —   | —         | Cast.    |
| F19                 | —    | —  | 98  | .12 | 1.0  | —    | .5  | —   | —         | Do.      |
| Cobalt-base alloys: |      |    |     |     |      |      |     |     |           |          |
| C1                  | 10   | 53 | 2   | —   | 20   | 15   | —   | —   | —         | Wrought. |
| C2                  | 1    | 65 | 1   | —   | 20   | 11   | —   | —   | —         | Cast.    |
| C3                  | 10.5 | 56 | —   | —   | 25.5 | 7.5  | —   | —   | 1.5 Cb.   | Wrought. |
| C4                  | —    | 57 | 1.5 | —   | 21   | 10   | —   | —   | —         | Cast.    |
| C5                  | —    | 67 | —   | —   | 20   | 12.5 | —   | —   | 8.0 Ta.   | Wrought. |
| C6                  | 2    | 62 | 1   | 5.5 | 27.5 | —    | —   | —   | —         | Cast.    |
| Nickel-base alloys: |      |    |     |     |      |      |     |     |           |          |
| N1                  | 54   | —  | 5.5 | 16  | 15.5 | 3.5  | —   | —   | —         | Wrought. |
| N2                  | 74   | —  | —   | 4.5 | 12.5 | —    | —   | —   | —         | Cast.    |
| N3                  | 61   | —  | 5   | 28  | —    | —    | —   | —   | —         | Wrought. |
| N4                  | 47   | —  | 18  | 9   | 22   | —    | —   | —   | —         | Cast.    |
| N5                  | 65   | —  | 9   | 5.3 | 15.5 | —    | —   | —   | 3 Al.     | Do.      |
| N6                  | 55   | —  | —   | —   | —    | 45   | —   | —   | —         | Wrought. |
| N7                  | 62   | 15 | —   | 3   | 10   | —    | —   | —   | 5.5Al5Ti. | Cast.    |
| Copper:             |      |    |     |     |      |      |     |     |           |          |
| M4                  | —    | —  | —   | —   | —    | —    | —   | —   | Cu.       | Wrought. |

The charge material is a crushed or shotted prealloyed aluminum alloy compound of the indicated materials. More specifically the charge material includes alloys of from about 19 to about 35 percent by weight aluminum and the balance substantially all iron and incidental impurities; alloys of from about 19 to about 35 percent by weight aluminum and the balance substantially all cobalt and incidental impurities; and alloys of from about 19 to about 35 percent aluminum and the balance substantially all iron and cobalt and incidental impurities. Specific and preferred charge material compositions are 30 percent aluminum-70 percent iron including incidental impurities and 30 percent aluminum-35 percent cobalt-35 percent iron including incidental impurities.

The charge material is of a size passing a No. 2 mesh sieve and held on a No. 50 mesh sieve. The preferred charge material consists of that material passing a No. 4 mesh sieve and held on No. 20 mesh sieve—the sieve sizes being those of the United States Standard Screen Series. With the use of these large particle sizes there is no problem of sintering of the charge material to the article to be coated as occurs when smaller sized charge material particles are used.

A chemical material, included in the retort with the charge material and article to be coated, is designated a carrier material for the purposes of this description because it is believed to bring the coating elements to the surface of the article to be coated. This material may be one or more of the halides of ammonium or aluminum. Preferred carrier materials are aluminum chloride, ammonium fluoride, ammonium chloride, ammonium bromide, and ammonium iodide. Aluminum chloride is the carrier material used in the preferred embodiment of the invention with the preferred charge material of 30 percent aluminum-70 percent iron alloy. The proportion of carrier material to charge material is from about 0.25 percent to about 3 percent by weight carrier material and from about 97 percent to about 99.75 percent by weight aluminum alloy charge material.

The heating step of the process is conducted at a temperature between about 1400° F. and 2000° F. for a time depending on the thickness of the coating intended. The thickness of the alloy coating can be varied by varying the time or temperature of the heating step.

In the drawing of the heating retort, FIG. 2, a heat resistant retort 11 is fitted with an encircling channel-shaped flange 12. Cover 13 fits over the retort with its sides 14 in the channel leaving space 15. A suitable sealing material 16 such as a fusible silicate or glass is placed in this space so that on heating of the retort, the glass melts to form a liquid seal allowing the escape of air from the retort. Contained in the retort is the charge material 17 of particulated aluminum alloy in which

are embedded several parts 18 to be coated. Under the charge material is a layer 19 of the selected carrier material. Those parts 20 which have internal cavities 21 to be coated are given an addition of carrier material 19 inside the cavity. After the retort and its contents have been heated and the reaction is complete, the retort is allowed to cool. The liquid seal material hardens forming a solid seal preventing the influx of contaminating air into the retort while the contents cool.

In operation when the retort and its contents are heated, it is believed that the halogen carrier volatilizes driving out the air from the retort through the liquid seal; the gaseous carrier reacts with the aluminum alloy charge material to form volatile metal halides; these compounds decompose at the surface to be coated depositing the coating elements and liberating the halogen which is then free to again enter into the coating process by reacting with the charge material.

The composition and characteristics of the diffused coating vary with the composition of the charge material. By the use of the indicated aluminum alloy charge materials in the ranges specified, superior coatings are produced. Because of equilibrium conditions set up in the retort at the surface of article to be treated and the indicated charge materials, alloy coatings are produced of definite and superior oxidation and erosion resistance. No filler materials or adsorbents are required in the charge material here, as in other processes.

Table 2 shows the coatings produced on different alloy articles using various charge material alloy compositions. The carrier material was ammonium fluoride and the heating conditions were 16 hours at approximately 2000° F. as shown. The alloy articles were of the same shape and size.

TABLE 2  
Effect of Charge Material Compositions

| Charge material | Alloy coated | Coating temp., ° F. | Coating thickness, mils | Coating characteristics  |
|-----------------|--------------|---------------------|-------------------------|--------------------------|
| 30 Al-70 Fe     | C2           | 2,000               | 3                       | Smooth and bright.       |
| 50 Al-50 Fe     | N2           | 1,950               | 5.4                     | Do.                      |
| 35 Co-35 Fe     | C2           | 2,000               | —                       | Articles badly corroded. |
| 30 Al           | N2           | 2,000               | 2                       | Do.                      |
|                 | N2           | 2,000               | 6.5                     | Smooth and bright.       |

As seen in Table 2 the charge material composition must be kept within the indicated ranges. A 50 percent aluminum-50 percent iron alloy charge material does not produce a satisfactory coating and in fact results in a

corrosive attack by the deposited metal on the article. It is only with the use of an alloy charge material containing from about 19 to about 35 percent aluminum and the balance, in this case, iron that the superior coating compositions of this invention are produced.

By means of X-ray diffraction analysis and X-ray fluorescence analysis of the alloy surface coated using the 70 Fe-30 Al charge material it was determined that the surface of the coatings of this invention were composed essentially of the intermetallic compound FeAl. This was true even when coating those nickel and cobalt-base alloy articles which did not contain any iron, thereby, demonstrating that iron and aluminum are co-deposited when the 70 Fe-30 Al charge material is used. These FeAl containing coating compounds give the high oxidation resistance and adherent bonding shown in the tables of oxidation and strength tests following. It was also demonstrated by X-ray analysis that there was no FeAl deposited when the charge material composition consisted of other iron-aluminum alloys outside the ranges of this invention. For example, the 50 percent by weight aluminum-50 percent by weight iron charge material produced the irregular coatings noted in Table 2, which coatings contained only aluminum and not FeAl, as demonstrated by X-ray analysis.

The minimum temperature of the heating step is about 1400° F. because at temperatures below 1400° F., the diffusion rate is too low. Actually the minimum temperature is determined by the decomposition temperature of the carrier compounds; and although the ammonium chloride decomposes at 662° F., and the aluminum chloride sublimes at 352° F., the lower temperature limit is set at 1400° F. for effective coating and diffusion in commercial production processing.

The thickness of the coating produced depends on several variables including time and temperature and these may be varied depending on the intended application. Generally, a heating time of from about 8 hours to 24 hours or more will produce a coating. For example, in FIG. 3, the iron base article was given a 10 mils thick coating by a heating at 1850° F. for 16 hours. In FIG. 4 the same alloy was given a 4.2 mils thick coat by reducing the heating temperature to 1600° F. for the same period of time.

In Table 3 the effects on the coating thickness of carrier material, process time, and temperature variations are shown. In each case the alloy charge material consisted of a 30 percent aluminum-70 percent iron composition and the carrier material was as indicated in the proportion of 0.5 percent carrier material and 99.5 percent charge material. The dimensional change resulting from the coating application is generally an increase in dimensions of about one half of the coating thickness applied.

TABLE 3  
Effect of Time and Temperature Variations on Coating Thickness  
FOR ALLOY C2

| Alloy Coated | Time, hours | Temperature, ° F. | Carrier                 | Coating Thickness, mils |
|--------------|-------------|-------------------|-------------------------|-------------------------|
| C2-----      | 16          | 1,850             | AlCl <sub>3</sub> ----- | 2.2                     |
| C2-----      | 24          | 1,800             | AlCl <sub>3</sub> ----- | 2.25                    |
| C2-----      | 24          | 1,900             | AlCl <sub>3</sub> ----- | 2.75                    |
| C2-----      | 16          | 2,000             | AlCl <sub>3</sub> ----- | 3.25                    |
| C2-----      | 64          | 1,950             | AlCl <sub>3</sub> ----- | 5.00                    |
| C2-----      | 8           | 1,400             | AlCl <sub>3</sub> ----- | 2.5                     |
|              | 5           | 1,700             |                         |                         |
| C2-----      | 9           | 2,000             | AlCl <sub>3</sub> ----- | 1.8                     |
|              | 20.6        | (1)               |                         |                         |

TABLE 3—Continued  
Effect of Time and Temperature Variations on Coating Thickness

OTHER ALLOYS

|    | Alloy Coated | Time, hours | Temperature, ° F. | Carrier                                       | Coating Thickness, mils |
|----|--------------|-------------|-------------------|-----------------------------------------------|-------------------------|
| 10 | F1-----      | 8           | 1,400             | AlCl <sub>3</sub> -----                       | >50                     |
|    | C1-----      | 5           | 1,700             | AlCl <sub>3</sub> -----                       | 1.9                     |
|    | C3-----      | 9           | 2,000             | AlCl <sub>3</sub> -----                       | 2.5                     |
|    | C4-----      | 16          | 1,600             | AlCl <sub>3</sub> -----                       | 3.0                     |
|    | N1-----      | 24          | 1,850             | AlCl <sub>3</sub> -----                       | 3.3                     |
| 15 | F4-----      | 24          | 1,850             | AlCl <sub>3</sub> -----                       | 20.0                    |
|    | N2-----      | 24          | 1,850             | AlCl <sub>3</sub> -----                       | 27.5                    |
|    | F15-----     | 24          | 1,850             | AlCl <sub>3</sub> -----                       | 12.5                    |
|    | F16-----     | 24          | 1,850             | AlCl <sub>3</sub> -----                       | 12.0                    |
|    | F17-----     | 24          | 1,850             | AlCl <sub>3</sub> -----                       | 20.0                    |
|    | F15-----     | 16          | 1,950             | NH <sub>4</sub> F plus NH <sub>4</sub> I----- | 7.0                     |
|    | F16-----     | 16          | 1,950             | NH <sub>4</sub> F plus NH <sub>4</sub> I----- | 9.0                     |
|    | F17-----     | 16          | 1,950             | NH <sub>4</sub> F plus NH <sub>4</sub> I----- | 8.5                     |
| 20 | F18-----     | 16          | 1,950             | NH <sub>4</sub> F plus NH <sub>4</sub> I----- | 24.0                    |
|    | F19-----     | 16          | 1,950             | NH <sub>4</sub> F plus NH <sub>4</sub> I----- | 16.5                    |
|    | F3-----      | 16          | 1,950             | NH <sub>4</sub> F plus NH <sub>4</sub> I----- | 15.5                    |
|    | F10-A-----   | 16          | 1,950             | NH <sub>4</sub> F plus NH <sub>4</sub> I----- | 13.5                    |
|    | F9-----      | 16          | 1,950             | NH <sub>4</sub> F plus NH <sub>4</sub> I----- | 22.5                    |
|    | F10-----     | 16          | 1,950             | NH <sub>4</sub> F plus NH <sub>4</sub> I----- | 15.0                    |
|    | F11-----     | 16          | 1,950             | NH <sub>4</sub> F plus NH <sub>4</sub> I----- | 12.0                    |
| 25 | F12-----     | 16          | 1,950             | NH <sub>4</sub> F plus NH <sub>4</sub> I----- | 2.0                     |
|    | F13-----     | 16          | 1,950             | NH <sub>4</sub> F plus NH <sub>4</sub> I----- | 1.25                    |
|    | C2-----      | 16          | 1,950             | NH <sub>4</sub> F plus NH <sub>4</sub> I----- | 2.5                     |
|    | C2-----      | 16          | 1,950             | NH <sub>4</sub> F-----                        | 2.6                     |
|    | C3-----      | 16          | 1,950             | NH <sub>4</sub> F-----                        | 1.9                     |
|    | C1-----      | 16          | 1,950             | NH <sub>4</sub> F-----                        | 3.7                     |
|    | N3-----      | 16          | 1,950             | NH <sub>4</sub> F-----                        | 3.4                     |
|    | N1-----      | 16          | 1,950             | NH <sub>4</sub> F-----                        | 2.5                     |
| 30 | N4-----      | 16          | 1,950             | NH <sub>4</sub> F-----                        | 2.8                     |
|    | N5-----      | 16          | 1,950             | NH <sub>4</sub> F-----                        | 3.8                     |
|    | F14-----     | 16          | 1,950             | NH <sub>4</sub> F-----                        | 4.2                     |
|    | N6-----      | 16          | 1,950             | NH <sub>4</sub> F-----                        | 3.5                     |
|    | N2-----      | 16          | 2,000             | NH <sub>4</sub> F plus NH <sub>4</sub> I----- | 2.9                     |
|    | C2-----      | 16          | 2,000             | AlCl <sub>3</sub> -----                       | 3.5                     |
| 35 | N2-----      | (2)         | 2,000             | AlCl <sub>3</sub> -----                       | 12.0                    |
|    | F4-----      | (2)         | 2,000             | AlCl <sub>3</sub> -----                       | 19.0                    |
|    | M4-----      | 6           | 1,400             | AlCl <sub>3</sub> -----                       |                         |
|    |              | 4           | 1,650             | AlCl <sub>3</sub> -----                       |                         |
|    |              | 6           | 1,850             | AlCl <sub>3</sub> -----                       |                         |

40 1 Continuous heating from room temperature to 2000° F.

2 Constant heating to 2000° F.

45 As seen in Table 3, the temperature requirements vary according to the desired coating thickness, alloy to be coated, and carrier material used. Table 3 shows the effects of time and temperature variations on the C2 alloy and also shows the rate of coating deposition for various other alloys. With information of this type a specific heating process can be designed to give a coating thickness of from about 1 mil to over 25 mils on a given alloy.

50 The temperature conditions can be varied as shown in Table 3 to meet a production operation. The heating can be done in a continuous sequence from room temperature to a temperature between about 1400° F. and 2000° F. for the length of time that is equivalent to a heating at a constant temperature between 1400° F. and 2000° F. The heating may also be conducted in stages for several hours at one temperature followed by heating for several more hours at another temperature. The times and temperatures for these operations are governed by the specific operating conditions and need only be at least equivalent to a heating at a temperature between about 1400° F. and 2000° F. for a time sufficient to form an effective coating.

65 A preferred heating cycle consists of placing the retort with contained articles and reactants in a furnace having an entry temperature of about 600° F. and an exit temperature of 2000° F. with a travel time of 24 hours—the temperature being raised from 600° F. to 2000° F. in about 20 hours.

70 As an example of the practice of the invention, the following description of the preparation of the prealloyed charge material is given. This material may be prepared

by several methods, such as powder metallurgical methods, etc., but alloying by fusion is preferred. In an induction furnace melting operation commercially available electrolytic iron (about 99.8 percent iron) and commercially available aluminum shot (about 99 percent aluminum) were used as raw materials in the proportion of 70 percent by weight iron and 30 percent by weight aluminum. The iron was melted first in a magnesia-lined crucible at a temperature of about 2950° F. Aluminum was added to the molten iron in batches of about 10 percent of the total required aluminum to avoid the undesirable effects of an overly exothermic reaction. After all of the aluminum was added, the melt was covered with a slag to prevent oxidation and volatilization of the aluminum and to permit interalloying. An inert atmosphere blanket may also be used for this purpose. The alloy was then shotted, washed in water, and dried.

The shot was then crushed in a jaw crusher to a size passing a No. 4 mesh sieve and held on a No. 20 mesh sieve. In other diffusion coating processes a much finer material is used with a resulting dust problem and the possible inclusion of fine particles in the coating because of sintering. The shot had the actual and intended composition shown in Table 4. The incidental impurities contained in the alloy do not interfere with the coating process. In fact, it must be noted the charge materials need not be made from ultrapure metal sources but rather may be commercially available iron and aluminum, for example, provided these sources do not contain an impurity content which interferes with the process.

TABLE 4

Composition in Weight Percent

|           | Desired | Actual  |
|-----------|---------|---------|
| Aluminum  | 30.0    | 29.56   |
| Iron      | Balance | Balance |
| Carbon    | Low     | 0.03    |
| Nickel    | Low     | 0.46    |
| Magnesium | Low     | nil     |
| Silicon   | Low     | 0.03    |
| Calcium   | Low     | nil     |
| Chromium  | Low     | 0.03    |

Other compositions of charge materials are made similarly using electrolytic cobalt, or other commercially available forms, when cobalt is part of the prealloyed charge composition.

When the charge material is cobalt-aluminum, the cobalt is first melted and then the aluminum added to the molten cobalt in several small additions.

When the charge material is iron-cobalt-aluminum alloy, the cobalt and iron are first melted together and then the aluminum additions are made.

It is to be noted that no catalysts, fillers, or adsorbents are used with the aluminum alloy charge material. A getter, such as titanium, may be used to remove oxygen in which case up to about 2 percent by weight of the total charge material would be powdered titanium metal mixed with the charge material.

The articles to be coated are first cleaned by any of the usual methods, such as grit blasting. The articles are then packed within the charge material in the retort with at least enough space between each article to allow for a layer of charge material. Cavities which are to be coated are charged with carrier material and with charge material. The remainder of the carrier material need not be mixed with the charge material (but may be so mixed) and can be placed at the bottom of the retort. This separate layer of carrier material on the floor of the retort heats more

quickly and volatilizes to purge the system of air and begin the coating action earlier than when the carrier agent is intermixed with the charge material. From about 0.5 to 1 percent by weight carrier material to about 99 to 99.5 percent charge material is generally used.

It is important to note that the articles to be treated need not be composed entirely of the same metal. Composite articles made of various nickel, iron and cobalt alloy parts may be successfully treated by this process. In one example, a jet engine component having parts made of four different alloys was coated in its assembled form. The article was composed of parts of two different cobalt alloys and two different stainless steels as well as various welding alloys. The coating was smooth and continuous over the entire article.

The loaded retort is heated at the temperature and for the time necessary to give the desired coating on the article to be coated. After the heating cycle is completed, the retort is cooled to a safe handling temperature. The coated objects are then removed and washed. They have a smooth, uniform, and continuous surface, even on hard-to-coat articles such as hollow blades and vanes. Additionally the coating on the inner surface of such hollow articles is equivalent in properties to that on the exterior surface.

The crushed charge material may be reused. In a series of tests a single batch of crushed 70 percent iron-30 percent aluminum alloy charge material was used ten times and was still usable. Only a washing with water and a screening to remove fine, exhausted particles is required before each reuse. After a large number of reuses the charge material may change in composition to an extent requiring either replacement or replenishment by remelting the depleted charge material and adding more pure metal.

Coated and uncoated specimens of the alloys were subjected to oxidation tests as a means to evaluate the improvement of the high-temperature properties effected by the coatings of this invention. The following oxidation test was used: specimens were weighed and then placed in a furnace operating at high temperature; moving dry air was continuously passed over the specimens; at the end of the testing time or at regular intervals, the specimens were removed from the furnace and again weighed and the weight change recorded. The weight change is a measure of oxidation resistance. Severe weight losses are an indication of heavy oxidation and consequent metal oxide spalling, while large weight gains result from the formation of massive metal-compound scales on the specimen surface. Optimum oxidation resistance is indicated when the specimen undergoes only slight weight changes and little or no spalling.

The articles to be tested were disc samples about  $\frac{3}{4}$  inch in diameter and  $\frac{1}{4}$  inch thick with  $\frac{1}{16}$  inch central hole. They were composed of the nickel, cobalt, and iron base alloys indicated in Tables 5 and 6. Some of these articles were coated according to the process of this invention while an equal number were left uncoated. The coating was produced by embedding the articles in a charge material of 30 percent aluminum-70 percent iron alloy with an aluminum chloride carriage agent in the amount of 99.5 percent charge material and 0.5 percent carrier material. The heating was carried out at about 1950° F. for 16 hours.

The oxidation tests were carried out at 2000° F. for 500 hours for the nickel and cobalt-base articles and at 1800° F. for 100 hours for the iron-base articles. In some cases weighing was made several times during the test as shown in the tables. The weight change is measured as mg. per cm.<sup>2</sup>.

9  
TABLE 5  
Results of Oxidation Tests at 2000° F. for 500 Hours

| Alloy No. | Weight change, mg./cm. <sup>2</sup> |          |          |          |          |          |          |          |
|-----------|-------------------------------------|----------|----------|----------|----------|----------|----------|----------|
|           | 20 hrs.                             |          | 100 hrs. |          | 300 hrs. |          | 500 hrs. |          |
|           | Coated                              | Uncoated | Coated   | Uncoated | Coated   | Uncoated | Coated   | Uncoated |
| C2.....   | +0.13                               | +0.82    | +0.72    | -41.27   | +1.12    | -147.46  | +1.2     | -200     |
| C3.....   | +0.54                               | -6.75    | +1.18    | -19.0    | +1.57    | -50.0    | +1.3     | -159     |
| N2.....   | +0.23                               | +0.42    | +0.43    | -0.69    | +1.08    | -3.33    | +0.1     | -3       |
| N3.....   |                                     |          |          |          |          |          | -11.2    | -372     |
| N5.....   |                                     |          |          |          |          |          | +1.0     | -37      |
| N6.....   |                                     |          |          |          |          |          | +2.7     | -60      |
| C2.....   |                                     |          |          |          |          |          | +4.0     | -474     |
| N2.....   |                                     |          |          |          |          |          | -0.04    | -3       |

TABLE 6  
Results of Oxidation Test at 1800° F. for 100 Hours

| Alloy No. | Weight change, mg./cm. <sup>2</sup> |          |         |          |         |          |          |          |
|-----------|-------------------------------------|----------|---------|----------|---------|----------|----------|----------|
|           | 49 hrs.                             |          | 66 hrs. |          | 83 hrs. |          | 100 hrs. |          |
|           | Coated                              | Uncoated | Coated  | Uncoated | Coated  | Uncoated | Coated   | Uncoated |
| F15.....  | +5.61                               | +215.7   | +5.86   | +238.9   | +6.02   | +230.9   | +7.5     | +262.4   |
| F15.....  |                                     |          |         |          |         |          | +4.1     | -203.7   |
| F16.....  | +2.40                               | -19.29   | +1.64   | -19.03   | +1.55   | -19.88   | +1.1     | -20.8    |
| F16.....  |                                     |          |         |          |         |          | +3.7     | -1.9     |
| F17.....  | +1.69                               | -1.89    | +1.64   | -2.02    | +1.60   | -2.45    | +1.5     | -3.3     |
| F17.....  |                                     |          |         |          |         |          | +4.7     | -18.4    |

The oxidation test results of Tables 5 and 6 show that both the coated and the uncoated specimens first underwent a weight gain as an initial layer of oxide formed. Spalling soon occurred on the uncoated specimens and net weight losses resulted, while the oxide layers on the 40 coated specimens were more protective and the rate of attack was at a very low level.

In another test coated and uncoated specimens of a C2 alloy article were heated to a temperature of 2300° F. in dry air. At the end of 4 hours, the uncoated specimens had lost an average of 141 mg./cm.<sup>2</sup> whereas the 45 coated specimens were unchanged. Further, at the end of 20 hours the coated specimens had gained only about 1.2 mg./cm.<sup>2</sup>.

These tests demonstrate that the coatings of this invention are quite effective in reducing the oxidation rate of iron, nickel, and cobalt-base alloys. The tests also show that the coatings are protective at temperatures approaching the melting points of the base alloy. It is to be understood that since the coating elements alloy with the base metal, the oxidation resistance of a coated article is somewhat dependent on the characteristics of the base metal. For example, it is seen that the coated nickel and cobalt base articles show a greater oxidation resistance than the coated iron-base articles.

A series of thermal shock tests were conducted in a special testing device. Specimens of coated and uncoated articles were automatically rotated to alternately hot and cold stations. At the hot stations, the specimens were heated by an oxyacetylene flame for seven seconds to a temperature of about 1950° F. Then at the cold stations the specimens were cooled in a blast of compressed air for seven seconds to about 300° F. The coated and uncoated specimens were of Alloy No. C2. Four uncoated specimens and four coated specimens were tested. After each 50 cycles of the above-described test, the specimens were removed and examined at 120 diameters magnification for cracks. The uncoated articles showed considerable cracks at 200 cycles and less while the coated specimens showed no cracks after 2000 cycles.

In an even more severe test the specimens were continuously exposed to an oxyacetylene flame for three 3-hour periods. A temperature of about 2050° F. was maintained on the specimens in this test with the weight change of the specimen used as the measure of the extent of the erosion. The coated specimens were coated in the same manner as in the previous tests. The results of this test are shown in Table 7 where it is seen that the uncoated specimens exhibited a metal loss while the coated 45 specimens developed a protective oxide film.

TABLE 7  
Flame Erosion Test Results

| Alloy No. | Weight change, mg./cm. <sup>2</sup> |          |         |          |         |          |
|-----------|-------------------------------------|----------|---------|----------|---------|----------|
|           | 3 hours                             |          | 6 hours |          | 9 hours |          |
|           | Coated                              | Uncoated | Coated  | Uncoated | Coated  | Uncoated |
| C2.....   | +0.7                                | +1.8     | +3.2    | -13.7    | +4.8    | -28.2    |
| C2.....   | +0.6                                | +1.1     | +3.3    | -56.2    | +4.6    | -57.4    |

The results of the several oxidation and erosion tests described above demonstrate that the diffusion coatings of this invention can be used in applications where high temperatures, aggressive environments, cyclic loads, thermal shock, or high velocity gas streams make the conventional alloys unsuitable for use or where coated articles of inexpensive alloys can be used in place of solid bodies of expensive, highly alloyed materials.

Additional tests were made to determine the mechanical properties of the coatings and to determine the effect of the coating process on the mechanical properties of the base alloy. Short time tensile tests were made on coated and uncoated specimens of Alloy No. C3 as shown in Table 8. The coated specimens were coated as before and tested as standard 1/4 inch tensile specimens.

TABLE 8

Average Tensile Test Results

| Test temperature, °F. | Condition | Ultimate tensile strength, p.s.i. | Yield strength 0.2% Offset, p.s.i. | Elongation in 1 inch, percent | Reduction of area, percent |
|-----------------------|-----------|-----------------------------------|------------------------------------|-------------------------------|----------------------------|
| Room                  | Coated    | 93,500                            | 70,400                             | 17.1                          | 9.8                        |
|                       | Uncoated  | 108,000                           | 76,200                             | 9.0                           | 11.0                       |
| 1,200                 | Coated    | 61,400                            | 36,000                             | 11.0                          | 12.9                       |
|                       | Uncoated  | 75,500                            | -----                              | 12.0                          | 12.6                       |
| 1,500                 | Coated    | 52,500                            | 32,400                             | 16.1                          | 18.7                       |
|                       | Uncoated  | 63,200                            | -----                              | 15.0                          | 18.5                       |
| 1,700                 | Coated    | 43,500                            | 29,100                             | 20.4                          | 26.0                       |
|                       | Uncoated  | 34,100                            | -----                              | 22.0                          | 35.8                       |
| 1,800                 | Coated    | 34,700                            | 20,800                             | 31.3                          | 40.9                       |
|                       | Uncoated  | 29,400                            | -----                              | 31.5                          | 38.8                       |

It is seen from the results of Table 8 that the coating had a relatively small influence on the tensile properties. The ultimate strength is lower than that of the uncoated alloy at 1500° F. and below. At higher temperatures, the ultimate strength of the coated specimens was slightly above the typical values of the uncoated alloy. The elongation of the alloy was not significantly affected by the coating. Generally, however, the yield and ultimate tensile strengths of the coated alloy are lower than those of the uncoated specimens of the same alloy while the elongation of the coated alloy is higher.

Charpy impact tests were conducted on coated and uncoated specimens of Alloy No. C2 at several temperatures using unnotched bars. Table 9 shows the results of these tests.

TABLE 9

Charpy Impact Strength of Coated and Uncoated Bars

| Test temperature, °F. | Condition | Charpy impact strength, ft.-lb. |     |         |
|-----------------------|-----------|---------------------------------|-----|---------|
|                       |           | High                            | Low | Average |
| Room                  | Uncoated  | 26                              | 18  | 23      |
|                       | Coated    | 32                              | 12  | 22      |
| 1200                  | Uncoated  | 77                              | 39  | 62      |
|                       | Coated    | 82                              | 38  | 58      |
| 1600                  | Uncoated  | 64                              | 43  | 56      |
|                       | Coated    | 60                              | 38  | 46      |
| 1800                  | Uncoated  | 54                              | 48  | 52      |
|                       | Coated    | 52                              | 35  | 40      |

The results of these tests show that the coated specimens generally exhibit a lower impact strength than the uncoated specimens but that the difference is relatively minor. More important is the fact that the coatings resisted spalling, cracking, and chipping under the most severe conditions of impact and deformation. In both the tensile tests and the impact tests conducted at temperatures of 1400° F. and above, the coating remained intact on the surface of the specimen, deforming with the base metal, even at the area of rupture. There was no spalling, flaking, or stripping of the coating, as is common with coating applied by other methods. This is attributable to the compatible ductilities of the coating and the base alloy. Additionally the coating is thoroughly diffused into the base object and becomes an integral part with the object, thereby eliminating the "layer effect" type of failure experienced by coatings applied by other methods.

It was also found that the hot hardness of a coated specimen was not significantly different from the hot hardness of the uncoated specimen. Additionally, it was found that the coated specimens exhibited a greater resistance to fatigue in many cases than the uncoated specimens as measured in rotating beam fatigue tests.

The coatings of this invention exhibit good resistance to attack by oil ash containing sulfur and vanadium compounds showing the usefulness of the coatings on hardware in furnaces burning residual fuel oils and in other similar applications.

It is seen that the coatings of this invention provide protection to metal particles from high temperature oxidation

and erosion attack, as well as thermal shock and mechanical fatigue and that the coating process does not significantly affect the strength of the base alloy but rather makes the base alloy suitable for use in more aggressive environments than originally possible. In addition, the high strength, adherence, and ductility of the coating allows for a thoroughly diffused and compatible bond with the base metal.

The above-described structural tests were conducted on iron, nickel and cobalt articles only, but oxidation tests were conducted on the diffusion coated copper M4 article shown in Table 4. The results of these tests are presented in Table 10.

TABLE 10

Results of Oxidation of M4 Alloy

[Same sample tested at each temperature]

| Temp., °F. | Time, hours | Unit weight change, mg./cm. <sup>2</sup> |          | Appearance            |                              |
|------------|-------------|------------------------------------------|----------|-----------------------|------------------------------|
|            |             | Coated                                   | Uncoated | Coated                | Uncoated                     |
| 1,200      | 4           | +0.32                                    | -13.7    | Retained luster.      | Discolored dull oxide scale. |
| 1,400      | 3           | +0.26                                    | -59.0    | Retained luster.      | Dull oxide scale.            |
| 1,600      | 3           | +0.70                                    | -106.6   | Retained luster.      | Dull oxide scale.            |
| 1,800      | 3           | +3.66                                    | -206.5   | Slight discoloration. | Heavy dull oxide scale.      |
| 30         |             | 1+4.94                                   | 1-385.8  |                       |                              |

<sup>1</sup> Total weight change.

It is seen that the diffusion coated copper articles show a significant improvement in oxidation resistance. Such coated articles are useful for applications requiring exposure to high temperatures, for example, blast furnace parts, electrical equipment, furnace fixtures, etc. Such parts, when uncoated, must be serviced or replaced periodically because of deterioration of the metal resulting from oxidation and subsequent scaling. The coating of this invention improves the oxidation resistance of these parts to a remarkable degree; consequently, the parts are less likely to fail or require periodic replacement.

The coating of this invention when applied to copper and copper-base alloys has a yellow color similar to pure gold. The combined properties of tarnish and oxidation resistance and a pleasing appearance makes this coating suitable for use on marine hardware and fixtures, decorative and other applications where an aesthetic quality is desired. For specific applications, a copper alloy with the desired physical and mechanical properties could be coated, thereby providing a novel article of manufacture.

What is claimed is:

1. A method for diffusion coating metallic articles comprising embedding the article to be coated in particulated, prealloyed charge material consisting essentially of from about 19 percent to about 35 percent by weight aluminum and the balance substantially all at least one metal selected from the group consisting of iron and cobalt and incidental impurities, and heating said charge material and contained articles in the presence of at least one carrier material selected from the group consisting of ammonium halides and aluminum halides, said heating being conducted with the exclusion of air at a temperature between about 1400° F. and 2000° F. for a time sufficient to form the coating.

2. A method for diffusion coating metallic articles composed of a material selected from the group consisting of iron-base alloys, nickel-base alloys, cobalt-base, and copper-base alloys comprising embedding the article to be coated in particulated, prealloyed charge material consisting essentially of from about 19 percent to about 35 percent by weight aluminum and the balance substantially all at least one metal selected from the group consisting of iron and cobalt and incidental impurities,

and heating said charge material and contained articles in the presence of at least one carrier material selected from the group consisting of ammonium halides and aluminum halides, said heating being conducted with the exclusion of air at a temperature between about 1400° F. and 2000° F. for a time sufficient to form the coating.

3. A method for diffusion coating metallic articles composed of a material selected from the group consisting of iron-base alloys, nickel-base alloys, cobalt-base alloys, and copper-base alloys comprising embedding the article to be coated in particulated, prealloyed charge material consisting essentially of from about 19 percent to about 35 percent by weight aluminum and the balance substantially all iron and incidental impurities, and heating said charge material and contained articles in the presence of at least one carrier material selected from the group consisting of ammonium halides and aluminum halides, the carrier material being present with the charge material in the relationship of from about 0.25 percent to about 3 percent by weight carrier material to from about 97 percent to about 99.75 percent charge material, said heating being conducted with the exclusion of air at a temperature between about 1400° F. and 2000° F. for a time sufficient to form the coating.

4. A method for diffusion coating metallic articles composed of nickel-base alloys comprising embedding the article to be coated in particulated, prealloyed charge material consisting essentially of from about 19 percent to about 35 percent by weight aluminum and the balance substantially all iron and incidental impurities, and heating said charge and contained articles in the presence of at least one carrier material selected from the group consisting of ammonium halides and aluminum halides, said heating being conducted with the exclusion of air at a temperature between about 1400° F. and 2000° F. for a time sufficient to form the coating.

5. A method for diffusion coating metallic articles composed of cobalt-base alloys comprising embedding the article to be coated in particulated, prealloyed charge material consisting essentially of from about 19 percent to about 35 percent by weight aluminum and the balance substantially all iron and incidental impurities, and heating said charge material and contained articles in the presence of at least one carrier material selected from the group consisting of ammonium halides and aluminum halides, said heating being conducted with the exclusion of air at a temperature between about 1400° F. and 2000° F. for a time sufficient to form the coating.

6. A method for diffusion coating metallic articles composed of copper-base alloys comprising embedding the article to be coated in particulated, prealloyed charge material consisting essentially of from about 19 percent to about 35 percent by weight aluminum and the balance substantially all iron and incidental impurities, and heating said charge material and contained articles in the presence of at least one carrier material selected from the group consisting of ammonium halides and aluminum halides, the carrier material being present with the charge material in the relationship of from about 0.25 percent to about 3 percent by weight carrier material to from about 97 percent to about 99.75 percent charge, said heating being conducted with the exclusion of air at a temperature between about 1400° F. and 2000° F. for a time sufficient to form the coating.

7. A method for diffusion coating metallic articles composed of a material selected from the group consisting of iron-base alloys, nickel-base alloys, cobalt-base alloys, and copper-base alloys comprising embedding the article to be coated in particulated, prealloyed charge material consisting essentially of about 30 percent by weight aluminum and the balance substantially all iron and incidental impurities, and heating said charge materials and contained articles in the presence of at least one carrier material selected from the group consisting of ammonium halides and aluminum halides, said heating

being conducted with the exclusion of air at a temperature between about 1400° F. and 2000° F. for a time sufficient to form the coating.

8. A method for diffusion coating metallic articles composed of nickel-base alloys comprising embedding the article to be coated in particulated, prealloyed charge material consisting essentially of about 30 percent by weight aluminum and the balance substantially all iron and incidental impurities and heating the charge material and contained articles in the presence of at least one carrier material selected from the group consisting of ammonium halides and aluminum halides, the amount of carrier material present with the charge material being in the relationship of from about 0.25 percent to about 3 percent by weight carrier material to about 97 percent to about 99.75 percent charge material, said heating being conducted with the exclusion of air at a temperature between about 1400° F. and 2000° F. for a time sufficient to form the coating.

9. A method for diffusion coating metallic articles composed of cobalt-base alloys comprising embedding the articles to be coated in particulated, prealloyed charge material consisting essentially of about 30 percent by weight aluminum and the balance substantially all iron and incidental impurities, and heating the charge material and contained articles in the presence of at least one carrier material selected from the group consisting of ammonium halides and aluminum halides, the amount of carrier material present with the charge material being in the relationship of from about 0.25 percent to about 3 percent by weight aluminum chloride to from about 97 percent to about 99.75 percent by weight charge material, said heating being conducted with the exclusion of air at a temperature between about 1400° F. and 2000° F. for a time sufficient to form a coating.

10. A method for diffusion coating metallic articles selected from the group consisting of iron-base, nickel-base, cobalt-base alloys, and copper-base alloys comprising embedding the article to be coated in particulated, prealloyed charge material of a particle size passing a No. 4 mesh sieve and held on a No. 20 mesh sieve, said charge material consisting essentially of from about 19 to about 35 percent by weight aluminum and the balance substantially all at least one metal selected from the group consisting of iron and cobalt and incidental impurities, and heating charge and contained articles in the presence of an aluminum chloride carrier material at a temperature between about 1400° F. and 2000° F. with the exclusion of air for a time sufficient to form a coating.

11. As a charge material for diffusion coating metal articles, a particulated alloy having a composition consisting essentially of from about 19 percent to about 35 percent by weight aluminum and the balance substantially all at least one metal selected from the group consisting of iron and cobalt and incidental impurities.

12. As a charge material for diffusion coating metal articles, a particulated alloy having a composition consisting essentially of from about 19 percent to about 35 percent by weight aluminum and the balance substantially all iron and incidental impurities.

13. As a charge material for diffusion coating metal articles, a particulated alloy having a composition consisting essentially of about 30 percent by weight aluminum and the balance substantially all iron and incidental impurities.

14. A metallic article having a protective coating of aluminum-containing, oxidation resistant materials formed by heating the article in a particulated, prealloyed charge material consisting essentially of from about 19 percent to about 35 percent by weight aluminum and the balance substantially all at least one metal selected from the group consisting of iron and cobalt and incidental impurities, said heating conducted in the presence of at least one carrier material selected from the group

consisting of ammonium halides and aluminum halides at a temperature between about 1400° F. and 2000° F. with the exclusion of air for a time sufficient to form the coating.

15. A metallic article having a protective coating of aluminum-containing, oxidation resistant materials formed by heating the article in a particulated, prealloyed charge material consisting essentially of from about 19 to about 35 percent by weight aluminum and the balance substantially all iron and incidental impurities, said heating conducted in the presence of at least one carrier material selected from the group consisting of ammonium halides and aluminum halides in an amount of from about 0.25 percent to about 3 percent by weight carrier material to about 97 percent to about 99.75 percent charge material, said heating conducted at a temperature of from about 1400° F. to 2000° F. with the exclusion of air for a time sufficient to form the coating.

16. A metallic article having a protective coating of

aluminum containing, oxidation resistant materials formed by heating the article in a particulated, prealloyed charge material consisting essentially of about 30 percent by weight aluminum and the balance substantially all iron and incidental impurities, said heating conducted in the presence of at least one carrier material selected from the group consisting of ammonium halides and aluminum halides at a temperature between about 1400° F. and 2000° F. with the exclusion of air for a time sufficient to form the coating.

References Cited in the file of this patent

UNITED STATES PATENTS

2,604,455 Reynolds et al. July 22, 1952  
15 2,657,129 Stern et al. Oct. 27, 1953

FOREIGN PATENTS

586,241 Great Britain Mar. 12, 1947  
812,301 Great Britain Apr. 22, 1959